

# UNITED STATES PATENT OFFICE.

FREDERIC LEWIS NATHAN, WILLIAM RINTOUL, AND FRANK BAKER, OF STEVENSTON, SCOTLAND, ASSIGNEES TO E. I. DU PONT DE NEMOURS POWDER COMPANY, OF WILMINGTON, DELAWARE, A CORPORATION OF NEW JERSEY.

## EXPLOSIVE.

1,090,643.

Specification of Letters Patent. Patented Mar. 17, 1914.

No Drawing.

Application filed June 4, 1913. Serial No. 771,622.

To all whom it may concern:

Be it known that we, FREDERIC LEWIS NATHAN, manager, WILLIAM RINTOUL, chief chemist, and FRANK BAKER, chemist, all of 5 Ardeer Factory, Stevenston, in the county of Ayr, Scotland, have invented a certain new and useful Improvement in and Relating to Explosives, and do hereby declare that the following is a full, clear, and exact de- 10 scription thereof.

This invention relates to the stabilizing of propellant explosives.

However carefully prepared, nitric esters, such as nitrocellulose, nitroglycerin, nitro- 15 mannite, and nitrostarch, undergo a slow decomposition even at ordinary temperatures, with the result that these substances, and mixtures containing one or more of them, are liable to deteriorate when kept 20 for considerable periods.

The products of the decomposition referred to, if allowed to remain in contact with the unchanged esters, exert an accelerating effect on the decomposition. Especially is this the case with explosives containing one or more members of the above mentioned class of chemical compounds, and such explosives are liable to become not merely unserviceable but dangerous. It is 30 therefore essential, in order to obtain an explosive of good chemical stability, that, besides being prepared from thoroughly stabilized materials, it shall have added to it some substances which will have the effect 35 of removing from it or rendering innocuous these products of decomposition.

It is already known that vaseline or mineral jelly exerts a stabilizing action on explosive into which it is introduced. It, however, possesses certain disadvantages which limit the stabilizing effects produced by it. For instance, it is an exceedingly complex substance, some of the components of it being very much less active in their stabilizing 45 properties than others. It is, however, entirely insoluble in nitroglycerin. These properties tend to produce a want of homogeneity in the explosive and ultimately to limit the stabilizing effect of this substance.

Again phenanthrene and diphenylamin have been proposed as stabilizing agents. These apparently possess the property of combining with the decomposition products of the nitric ester to form a nitro-compound

and one which possesses no accelerating ac- 55 tion on the inherent rate of decomposition of the ester. Although benzine, for instance, can be nitrated, it would be of little use as a stabilizer in explosives, not only because of its volatility but also because of the slowness 60 and difficulty with which its nitration is brought about. It is therefore evident that all substances which will nitrate are not necessarily stabilizers in the sense that they will materially prolong the life of explosive mix- 65 tures into which they are introduced.

We have found that in order that a substance may be an effective stabilizer, not only must it be capable of easy nitration with formation of a substance or of substances possessing no accelerating effect on the inherent rate of decomposition but moreover it must be capable of being homogeneously retained within the explosive in quantity sufficient to effect stabilization. 75

Separation of the stabilizer or its product of nitration from the powder when the latter is dried or afterward during storage, leads to alterations in the composition and ballistic properties of the explosive, and is therefore very undesirable. The stabilizer should for instance be soluble in nitroglycerin to such an extent that it will not separate out in this way. In cordite for example, containing 30 parts of nitroglycerin and 5 parts 85 of stabilizer, when it is desired to replace the mineral jelly which is the present stabilizer with one which would be homogeneously retained in solution in the nitroglycerin present, it would be necessary to select a 90 stabilizer which would remain in solution in the nitroglycerin to the extent of at least 16%.

Now we have further ascertained that there exist a large number of substances 95 which are capable of fulfilling the requirements indicated. These substances are compounds which have aromatic radicals readily undergoing nitration and which while producing stable compounds with the decomposition products of the nitric ester, are, moreover, homogeneously retained by nitric ester explosives in sufficient quantity to give efficient stabilization. Examples of these substances are chemical compounds of the class 100 known as ethers, or compounds of the constitution  $R-O-R'$  of which one or both of the radicals  $R$  or  $R'$  is an aromatic rad-

ical, such as phenyl, benzyl, naphthyl, phenanthryl, etc., or a homologue of them.

This invention consists therefore broadly in effecting stabilization of propellant explosives formed of or containing a nitric ester such as nitroglycerin or nitrocellulose by including therein one or more substances of the kind indicated in suitable quantity.

10 The following are examples of one class of the compounds referred to:—diphenyl-ether  $C_{12}H_{10}O$ , phenyl-benzyl-ether  $C_{13}H_{12}O$ , ethyl-naphthyl-ether  $C_{12}H_{12}O$ , and phenanthryl-methyl-ether  $C_{15}H_{12}O$ .

15 In judging which substance or substances is or are the most suitable for use in any particular case, we are guided by the properties of the individual compounds such as volatility, solubility in nitroglycerin, and 20 the readiness with which they become nitrated. As these substances are introduced into explosives with the view of absorbing the products of decomposition by becoming nitrated, their higher nitro-derivatives are 25 unsuitable for this purpose because of the increasing difficulty with which nitration occurs as the degree of nitration rises.

As an example of the use, according to 30 our present invention of one of the above class of compounds, an explosive of the following composition may be cited:—

|                        |     |
|------------------------|-----|
| Nitroglycerin          | 30% |
| Guncotton              | 65% |
| Ethyl-6-naphthyl-ether | 5%  |

The proportion of the stabilizer to be used according to our present invention may be

varied, according to the nature and proportions of the other components of the mixture in which it is used.

We are aware that similar compounds have been used in connection with pyroxylin which we do not claim herein.

We claim:

1. An explosive containing at least one 45 highly nitrated nitric ester and an ether containing an aryl group containing only carbon and hydrogen.

2. An explosive containing nitroglycerin, nitrocellulose and an ether containing an 50 aryl group containing only carbon and hydrogen.

3. An explosive containing nitroglycerin, nitrocellulose and ethyl & naphthyl ether.

4. An explosive containing gelatinized together at least one highly nitrated nitric ester and an ether containing an aryl group containing only carbon and hydrogen.

5. An explosive containing gelatinized together nitroglycerin, nitrocellulose and an 60 ether containing an aryl group containing only carbon and hydrogen.

6. An explosive containing gelatinized together nitroglycerin, nitrocellulose and ethyl & naphthyl ether.

In testimony that we claim the foregoing we have hereunto set our hands.

FREDERIC LEWIS NATHAN.  
WILLIAM RINTOUL.  
FRANK BAKER.

Witnesses:

M. B. MILNE,  
ERNEST HANSFORD.

Copies of this patent may be obtained for five cents each, by addressing the "Commissioner of Patents, Washington, D. C."